# EUROPEAN PATENT APPLICATION

(11) **EP 0 514 069 A1**
(43) Date of publication of application: **19.11.1992**
(21) Application number: 92304066.1
(22) Date of filing: 06.05.1992
(51) Int. Cl.: G03C 5/26

(54) **Concentrated developing solutions**

(30) Priority: 15.05.1991 GB 9110481
(71) Applicant: ILFORD Limited, Mobberley Knutsford Cheshire WA16 7JL (GB)
(72) Inventor: Parker, Michael John, Holmes Chapel, Crewe, Cheshire CW4 7LS (GB)
(74) Representative: Matthews, Richard Nordan

(57) **Abstract**

There is described a concentrated developing solution which comprises per litre of water 100 to 300g of sodium sulphite and from 50 to 150g of potassium sulphite the % by weight ratio of the sodium sulphite to the potassium sulphite being from 25:75 to 75:25, a total of from 30 to 50g of at least one silver halide developing agent, a buffering substance, sufficient sodium hydroxide to yield a pH of from 8.0 to 11.5 when the concentrated developer solution is diluted 1 plus 4 water, and as the sequestering agent from 5 to 40g of diethylene - triamine - pentaacetic acid.

It has been found that the choice of DTPA as the sequestering agent lower the resolution temperature of the developing solution. Thus the concentrated developing solution can be stored at a lower temperature than if other sequestering agents had been used.

## Description

This invention relates to silver halide material developing solutions.

There is a continuing need to provide new types of developing solutions as the commercial needs change. At the moment liquid concentrate developing solutions are finding greater favour than powder developers. That is to say, all the ingredients which are necessary to effect development of the exposed silver halide material are dissolved in an aqueous solution which is made as concentrated as possible. This solution is diluted with water to prepare a working strength solution.

Liquid concentrate developer solutions tend to suffer from the defect that storage of the solutions at well below ambient temperature causes the ingredients in the solution to precipitate. This of course negates the chief advantage of liquid concentrate developing solutions over powder developer mixtures. This is especially true if it is required to heat-up the liquid concentrate to cause the precipitated solids to dissolve. Concentration wise, the most important ingredient of liquid concentrate developers is the alkali metal sulphite which is always present. The sulphite may be present as potassium sulphite which is very soluble or as sodium sulphite which is not so soluble. Thus, if all the sulphite is present as potassium sulphite, the temperature required to redissolve the precipitated ingredients of a liquid concentrate developer, which has been stored at a temperature sufficiently low to cause such precipitations, is lower than if sodium sulphite had been present in the developer solution. The resolution temperature is defined as the temperature at which all precipitated solids re-dissolve on stirring following storage of the concentrated developer sample at -15°C. However, potassium sulphite is considerably more expensive than sodium sulphite. Further when the diluted liquid concentrate developer is used in a processing system wherein a fixing tank follows the developing tank a certain amount of the diluted developing solution is carried over from the developing tank to the fixing tank. Potassium salts present in the fixing solution tend to cause the fixing time to increase. Thus it is preferred that sodium sulphite is used in the developing solution.

Concentrated developing solutions comprise all the ingredients required to prepare a working developing solution when the concentrate is diluted. This is often 1 part of solution to 4 of water.

Most usually working developing solutions comprise a sequestering agent to sequester calcium, magnesium and iron ions thus preventing these substances forming sludges and precipitations in the developing tank or processing container. Unexpectedly, it has been found that the choice of the sequestering agent when present in the concentrated developer solution has a great effect on resolution temperature of the developing solution.

Therefore according to present invention there is provided a concentrated developing solution which comprises per litre of water 100 to 300g of sodium sulphite and from 50 to 150g of potassium sulphite the by weight % ratio of the sodium sulphite to the potassium sulphite being from 25:75 to 75:25, a total of from 30 to 50g of at least one silver halide developing agent, a buffering substance, sufficient sodium hydroxide to yield a pH of from 8.0 to 11.5 when the concentrated developer solution is diluted 1 plus 4 water, and as the sequestering agent from 5 to 40 g of diethylene - triamine - pentaacetic acid.

Diethylene - triamine - pentacetic acid is usually supplied as the free acid but when added to the concentrated developing solution becomes the sodium salt. However, the potassium salt could be added to the concentrated developing solution.

The sodium salt of diethylene - triamine - pentaacetic acid is hereinafter referred to as DTPA.

Preferably the concentrated developing solution comprises both a hydroquinone type developing agent, and most preferably hydroquinone itself, and a 1 - phenyl - 3 - pyrazolidinone developing agent of the general formula 1:-
wherein R₁ is hydrogen, methyl or ethyl, R₂ is hydrogen, methyl or -CH₂ OH and R₃ is hydrogen, methyl or ethyl.

Other useful hydroquinone type developing agents include chloro-hydroquinone, methyl hydroquinone and gentisic acid.

The preferred 1 - phenyl - 3 pyrazolidinone are the compound wherein R₁, R₂ and R₃ are all hydrogen and the compound wherein R₁ is methyl R₂ is - CH₂OH and R₃ is hydrogen.

Para-amino phenol type developing agents such as metol can be used instead of pyrazolidinone developing agents.

The preferred amount of hydroquinone type developing agent in the concentrated developing solution is from 20 to 60 g/litre.

The preferred amount of 1 - phenyl - 3 - pyrazolidinone developing agent or para-amino phenol type developing agent in the concentrated developing solution is from 1 to 10 g/litre.

Preferably sufficient buffering agent is present to buffer the diluted concentrated developing solution within a pH range of ± 1 pH unit of the chosen pH.

The preferred buffering agent is an alkali metal carbonate.

The preferred % by weight ratio of sodium sulphite to potassium sulphite present in the concentrated developing solution is 50% sodium to 50% potassium.

Thus in the concentrated developer solution of the present invention the ratio of sodium sulphite to potassium sulphite is so chosen that the resolution temperature is reduced as low as possible without using too much potassium sulphite which is more expensive than sodium sulphite and which can carry-over into the fixer bath and slow the rate of fixation. Using the ratio of sodium to potassium specified as shown in the example which follows the resolution temperature can be reduced as low as +3°C.

Preferably at least one so-called restrainer is present in the concentrated developing solution. This so-called restrainer serves to inhibit fog formation in the processing of exposed film in the diluted developing solution. Most preferably both an inorganic restrainer such as potassium bromide and an organic restrainer such as benzotriazole are present in the concentrated developing solution.

The following Example will serve to illustrate the invention.

### Example

In order to illustrate the effect of the type of sequestering agent used on the resolution temperature of a concentrated developer solution the following concentrated developer solutions were prepared.:-

The amount of sodium hydroxide was sufficient to yield a pH of 10.6 when the concentrated developer was diluted 1+4. The amount varied with the sequestering agent present in the solution as some of those used are very strongly acid. Solution 1 comprised diethylene - triamine - pentaacetic acid (DTPA).

Solution 2 comprised 1, 3-diamino - 2 - propanol-tetraacetic acid (DAPTA).

Solution 3 comprised 1 - hydroxyethylidene 1, 1 - diphosphonic acid which has the formula:
as a 60% by weight aqueous solution.

Solution 4 comprised pentasodium aminotri (methylphosphonate) which has the formula:-
as a 40% by weight aqueous solution.
Ethylene diamine tetraacetic acid (EDTA) which used to be used as a sequestering agent is now no longer used as when iron has been sequestered it acts as an oxidising bleaching agent and thus can cause adverse sensitometric effects when present in the developer solution.

The resolution temperatures of solutions 1 to 4 were as follows:-

This shows the remarkable lowering of the resolution temperature when DTPA is used as the sequestering agent compared with the use of other known sequestering agents.

In order to illustrate the effect of altering the sodium/potassium sulphite ratio the following concentrated developer solutions were prepared:-

5 variants of this were tested with the following results:-

Thus solution 1 had all sulphite present as the sodium salt
solution 2 had a sodium to potassium sulphite ratio of 75:25 by weight
solution 3 had a sodium to potassium sulphite ratio of 50:50 by weight
solution 4 had a sodium to potassium sulphite ratio of 25:75 by weight
solution 5 had all sulphite present as the potassium salt

Thus all the concentrated developer solutions according to present invention had a greatly reduced resolution temperature compared with the sodium sulphite solution.

Whilst the most preferred concentrated developer solution that is the solution wherein the ratio of sodium to potassium is 50:50 had a greatly reduced resolution temperature combined with a great reduction in the amount of potassium sulphite used.

## Claims

1. A concentrated developing solution which is characterised in that it comprises per litre of water 100 to 300g of sodium sulphite and from 50 to 150g of potassium sulphite the % by weight ratio of the sodium sulphite to the potassium sulphite being from 25:75 to 75:25, a total of from 30 to 50g of at least one silver halide developing agent, a buffering substance, sufficient sodium hydroxide to yield a pH of from 8.0 to 11.5 when the concentrated developer solution is diluted 1 plus 4 water, and as the sequestering agent from 5 to 40g of diethylene - triamine - pentaacetic acid.

2. A concentrated devloping solution according to claim 1 characterised in that wherein % by weight ratio of sodium sulphite to potassium sulphite present in the concentrated developing solution is 50% sodium to 50% potassium.

3. A concentrated developing solution according to claim 1 characterised in that it comprises both a hydroquinone type developing agent and a 1 - phenyl - 3 - pyrazolidone developing agent of the general formula 1:- wherein R₁ is hydrogen, methyl or ethyl, R₂ is hydrogen, methyl or -CH₂ OH and R₃ is hydrogen, methyl or ehtyl.

4. A concentrated developing solution according to claim 3 characterised in that the 1 - phenyl - 3 pyrazolidinone is the compound wherein R₁, R₂ and R₃ are all hydrogen and the compound wherein R₁ is methyl R₂ is - CH₂OH and R₃ is hydrogen.

5. A concentrated developing solution according to claim 3 characterised in that the amount of 1 - phenyl - 3 - pyrazolidinone developing concentrated developing solution is from 1 to 10g/litre.

6. A concentrated developing solution according to claim 1 characterised in that the amount of hydroquinone type developing agent in the concentrated developing solution is from 20 to 60g/litre.
